

Dec. 12, 1939.

C. W. HAGENBUCH ET AL

2,182,805

GRINDING BALL

Filed Dec. 15, 1937

*Fig. 1*



*Fig. 2*



INVENTORS  
CHARLES W. HAGENBUCH  
FREDERICK A. MC COY  
BY  
*Alfred R. Fuchs*  
ATTORNEY

## UNITED STATES PATENT OFFICE

2,182,805

## GRINDING BALL

Charles W. Hagenbuch and Frederick A. McCoy,  
Kansas City, Mo., assignors to Sheffield Steel  
Corporation, a corporation of Ohio

Application December 15, 1937, Serial No. 179,935

6 Claims. (Cl. 83—9)

Our invention relates to grinding elements for use in ball mills, and more particularly to a grinding ball, or slug, for use in such mills.

In the use of loose members that are adapted to grind by means of a combination of rolling, rubbing and pounding action, such as takes place in the type of pulverizing or grinding apparatus commonly known as a ball mill, various sizes of such loose grinding members, or elements, are utilized. These are ordinarily referred to as balls, even though the same may not be true spheres, and are sometimes referred to as slugs. The term "ball", as used herein, is not used in its narrow sense of "sphere", but in the sense in which it is used in the ball mill art, that is, to designate one of a collection of loose grinding elements, which are permitted to roll and tumble about in a suitable container, such as the drum or other container of a grinding mill.

It has been found desirable in ball mills, to use balls, or loose grinding elements, in the same mill, that are of various sizes, either by starting the mill with balls of different sizes therein, or by obtaining the smaller sized balls, or grinding elements, by the gradual wear of the elements from a standard starting size. After a ball mill has been started and is in operation for a period of time, there will be numerous sizes of the loose grinding elements in the mill, and it is only necessary to add the largest size elements, that are desirable to use in the mill, as these have to be replaced.

Ball mills are used for many purposes, in reducing materials, and are adapted for pulverizing many materials. Such mills are used for grinding materials in both a wet and a dry state. Ores and similar materials are usually in a wet state. In grinding materials that are dry, as for instance in the clinker mills in the manufacture of Portland cement, the materials are usually reduced or ground at a comparatively high temperature, due to the friction produced in grinding.

It is accordingly desirable, in making such loose grinding elements for ball mills, commonly referred to as grinding balls or slugs, to provide a member that will not wear too rapidly, and which will withstand the pounding action in the mill that results from the balls dropping from the upper portion of the mill to the lower portion thereof, and which will also not be materially altered in their physical characteristics by the heat that exists in a ball mill when certain materials are ground in a dry state.

Grinding balls have been made for many years of a hardened heat treated carbon-manganese alloy steel containing from .4 per cent to 1.2 per cent carbon. As large quantities of these grinding balls, or elements, are used in each ball mill in reducing ores at mines, and for similar purposes, the fact that these carbon-manganese

steel grinding balls of the above mentioned character wore rapidly, caused considerable unnecessary expense due to the necessity of purchasing and handling large quantities of these balls, or elements. The difficulty with a steel of the above mentioned character is, that when hardened sufficiently to reduce the rapidity of wear thereof, it becomes so brittle, that the tendency of the grinding ball, or element, to crack and flake off is considerably increased, and as a result there is no ultimate gain obtained by the hardening of such a grinding element beyond a certain stage. While it is desirable to increase the carbon content of steel alloy grinding elements, in order to increase the hardness thereof, yet if the carbon content is increased to the higher percentage limit mentioned above the proper ductility required for withstanding impact will not be present. It has been found by test that the finer the grain of the steel, having a certain hardness, the less the wear will be under the conditions existing in ball mills.

While various methods of heat treatment and of hardening have been utilized in the art, and the balls, or grinding elements, have been quenched in a bath of oil, or water, or other cooling medium, to harden the same, the effect on the grain structure and wearing qualities of the heat treatment and rapid cooling of the carbon-manganese steel alloy ball has been such in all cases that the life of the balls, or elements, was not as long as is desirable. Variations, of course, exist in the hardness, depending upon the quenching medium, temperatures and compositions used, but the final result, as far as wear is concerned, by the use of different cooling mediums, does not vary greatly, although we have found in practice, in hardening steels of the above mentioned character, that water gives better results, as far as wear and hardness are concerned, than other cooling baths that might be used.

It is a particular object of our invention to provide a grinding ball, or slug, that has very great wear resisting properties, and which is not very much more expensive to make than grinding balls, or slugs, made of carbon steel alloys, previously used for this purpose, so that, due to the much greater wearing qualities of our improved grinding element, a very great saving in cost of grinding members per ton of material operated on results from the use of our improved grinding elements. We have found that by using a molybdenum steel alloy for the grinding balls, we can use a higher carbon content in our improved grinding balls or elements than has been previously possible, and obtain a member that has great hardness, great wearing properties, and great resistance to breakage, due to the fact that the alloy develops a requisite amount

of ductility, and a very fine grain structure can be obtained by hardening, in a manner to be described, a ball or grinding element made of molybdenum steel alloy of the character that we utilize. Also, the ball or grinding element made of this alloy will not lose its hardness when used for grinding purposes in cement plant ball mills, due to the high temperature encountered therein; and materials that tend to adhere to the surface of the usual carbon-manganese steel balls and reduce the efficiency thereof will not adhere to our grinding elements to the same extent as to the carbon-manganese balls previously used, thus preventing uneven wear of the balls or grinding elements due to such adherence of the materials that are being ground to the surface of the ball at certain points.

While it has been known for many years that molybdenum increases the wearing qualities of steel, the molybdenum alloys previously known were not made for successful use in making grinding balls, or slugs, or grinding elements, to use in ball mills. It is, of course, to be appreciated that these grinding balls or elements cannot be made of an extremely expensive alloy, because these are constantly being used up and have to be constantly replaced in the mill. Even if such molybdenum alloys as were used for other purposes had been used in grinding balls, these balls would not have been satisfactory, because either the wearing qualities thereof would not have been sufficient to make the use thereof economical, or the first cost of these balls would have been so great that the increase in the wearing properties thereof would have been insufficient to overcome this increase in cost. An entirely different situation exists in making grinding balls than in making tools, or railroad rails, or other similar members, that are used for long periods of time.

Grinding balls of the most excellent wearing qualities could not have an extremely long life, because of the hard service to which the same are subjected. The wearing qualities of alloy steels, in which molybdenum has been previously used, have been attributed to the resistance to abrasion of the molybdenum itself. From this standpoint the greater the percentage of molybdenum used the greater the wearing properties of the alloy. For this reason it had been, prior to this invention, customary to keep the carbon content of molybdenum alloys relatively low and the molybdenum content relatively high, in order to increase the wearing properties, and obtain toughness.

We have discovered, however, that in a grinding ball or grinding element, molybdenum in the alloy used can serve an entirely different purpose. The presence of the molybdenum increases the wearing properties of the alloy, but it is not primarily due to the abrasion resisting properties of the molybdenum itself that increased wear and longer life in our grinding ball is obtained. The increase in wear and longer life is due to the fact that, by the use of molybdenum, we are able to control the grain structure by heat treatment and hardening of the ball, or grinding element, whereby we obtain a denser and finer grained steel than has been previously obtained in grinding balls. The finer grain structure that is obtained is coupled with a greater depth of hardening than has been previously obtainable in hardened steel grinding balls. As a result, a ball is produced that is hard and does not wear rapidly on its surface, and is not of a coarse grain structure, and yet is not so brittle that it

will chip off or crack under impact, such as exists under conditions present in many ball mills.

It is a particular purpose of our invention to provide a grinding ball of the above mentioned character that is made up of steel of very fine grain structure, in the martensitic state, which extends inwardly from the outer surface of the grinding ball or element to the center thereof in the case of small grinding balls or elements, and inwardly to substantially the center thereof in grinding balls of medium size, while in the case of grinding balls of the larger sizes, the fine grained martensitic structure of the steel extends inwardly to such a depth that the size of the grinding element or ball will have been reduced, in even the largest size balls, by substantially one-third the original diameter thereof, before the inner core of a coarser grain structure is reached. The inner core is, however, of a finer grain than is obtained by heat treatment and quenching of previously used carbon-manganese steel alloys, no matter what sort of heat treatment and cooling medium might have been used in carrying out the hardening process. The center of the core is largely troostite and sorbite, while an intermediate zone between the outer fine grained martensitic zone and the center of the core, comprises martensite, as well as troostite and sorbite, the core having more elasticity than the outer hard, dense, fine grained zone.

It is also a purpose of our invention to provide a new and improved method of making a grinding ball or element, whereby a grinding ball or element having the aforementioned desirable characteristics is produced.

Other objects and advantages of our invention will appear as the description of the drawing proceeds. We desire to have it understood, however, that we do not intend to limit ourselves to the particular details shown or described, except as defined in the claims.

#### In the drawing:

Fig. 1 is a transverse sectional view through a grinding ball of relatively large diameter, made in accordance with our invention, showing the grain structure, and

Fig. 2 is a similar sectional view of a small grinding ball, made in accordance with our invention.

In making our improved grinding member, a molybdenum steel alloy is used, which, preferably, contains carbon, manganese, molybdenum, and silicon or aluminum, within the percentage limits below set forth:

|                     | Per cent    |
|---------------------|-------------|
| Carbon              | .60 to 1.10 |
| Manganese           | .30 to 1.10 |
| Molybdenum          | .10 to .80  |
| Silicon or aluminum | Up to .30   |

The remainder of the alloy is iron, except for extremely small percentages of impurities that exist in the iron.

For certain uses it is desirable to produce a grinding element that will not corrode or rust, and we prefer to include from .20% to .30% copper in the alloy to retard corrosion or rusting, in addition to the above referred to ingredients, within the percentage limits mentioned herein, when the grinding elements are to be used under conditions in which rusting or corrosion might take place.

As a specific example of an alloy found highly desirable and giving the desired grain structure, hardness and wearing properties for a grinding

|                                                             | Per cent |
|-------------------------------------------------------------|----------|
| Carbon                                                      | .70      |
| 5 Manganese                                                 | .60      |
| Silicon, not over                                           | .25      |
| Molybdenum                                                  | .20      |
| Iron, not less than                                         | 98.00    |
| 10 Impurities, mainly sulphur and phosphorus, approximately | .25      |

The grinding element is formed in any desired manner into the shape desired, which may be referred to as a ball or slug, and which is usually spherical, although not necessarily so, but forging is found to be preferable because greater homogeneity of the grinding ball or element appears to be obtainable by forging than by casting. The grinding ball after being shaped is heat treated, preferably, by heating to a temperature of approximately 1450 degrees F. After the grind element attains the desired temperature it is quenched in a cooling medium for a sufficient period of time to reduce the temperature of the grinding ball to approximately 200 degrees F., after which it is cooled, in the atmosphere, to atmospheric temperature at a rate of not to exceed 200 degrees F. per minute. The quenching can be done in water, oil, or brine, as may be found preferable. When a ball one-half inch in diameter is quenched in water, the ball is completely immersed in the water for five seconds, the water being at a temperature between 80 and 90 degrees F. Instead of heating the grinding ball after it has been forged to shape, it may be quenched in the quenching medium, in the case of small sized balls, immediately after forging the same, before it cools, without re-heating, but in that case, the manganese content of the ball is, preferably, reduced below that above mentioned.

40 While the composition above mentioned is preferred for a ball one-half inch in diameter that is quenched in water, some variation from this composition can be used and yet approximately the same results can be gotten as with the preferred composition. Thus the carbon content can be varied between .60% and .85%, the manganese content can be varied between .45% and .65%, if re-heated, and between .35% and .55%, if quenched directly after forging, and the molybdenum content can be varied between .10% to .20%, and the silicon content can be varied between .10% to .25%, and grinding balls of such small diameter as one-half inch produced, that have the desirable characteristics and length of life that form the principal advantages of our improved grinding elements. Of course, if it is desired to produce a rust or corrosion resisting ball from .20% to .30% copper can be added to the composition, or even higher percentages of copper can be added, if it is desired to not only provide rust or corrosion resisting properties, but additional strength by means of copper in the alloy.

As the diameter of the balls increases, it is found to be desirable to increase the carbon content to obtain these desirable characteristics. Thus, for example, a ball three-fourths inch in diameter, preferably, contains from .60% to .90% carbon; a one inch ball, preferably, contains from .62% to .95% carbon; a one and one-half inch ball from .62% to .95% carbon; a two inch ball from .62% to 1.00% carbon; a three inch ball from .65% to 1.00% carbon; a four inch ball from .70% to 1.05% carbon; a five inch ball from .70% to 1.05% carbon, while a ball ten inches in di-

ameter will, preferably, have from .75% to 1.10% carbon.

The character of the quench used determines to a certain extent the amount of carbon that should be present in the alloy. Thus a brine quench will require the lowest percentage of carbon, and an oil quench the highest percentage. Thus for the one-half inch balls, preferably, the carbon content of a ball that is to be oil quenched is from .75% to .85%; for a ball to be water quenched, from .65% to .75%, and for a ball to be brine quenched, from .60% to .70%.

The temperature to which the ball is heated before quenching is also varied in accordance with the quench used. Thus for a brine quench the temperature at which the ball is quenched is from 1425 degrees F. to 1450 degrees F., whereas for a water quench it is from 1450 to 1500 degrees F., and for an oil quench, from 1500 to 1550 degrees F., for a one-half inch ball. The quenching temperature also gradually rises with the size of the ball, and for a five inch ball the quenching temperatures are substantially 125 degrees F. to 175 degrees F. more than for a one-half inch ball. Also the quenching time required increases gradually with the size of the ball. For example, when a water quench is used the time required for quenching the one-half inch ball is five seconds; the three-fourths inch ball ten seconds; the one inch ball eighteen seconds; the two inch ball forty-two seconds, the three inch ball eighty seconds and the five inch ball one hundred and ten seconds.

The manganese content of the balls varies with the size of the ball and also is dependent upon the manner in which quenching is done. If the balls are allowed to cool in the atmosphere and are re-heated and then quenched a higher percentage of manganese can be used without causing internal stresses in and brittleness of the balls, than if the quenching is done directly after the ball is forged. Thus a one-half inch diameter, water quenched ball that has been allowed to cool and is re-heated may have a manganese content varying between .45% and .65%; a one inch water quenched ball, similarly treated, a manganese content varying between .50% and .60%, and a three inch water quenched ball, similarly treated, a manganese content varying between .55% and .75%, and an oil quenched ball of one-half inch diameter, similarly treated, may have a manganese content varying between .55% and .75%, a one inch oil quenched ball, similarly treated, a manganese content varying between .65% and .85%, and a three inch oil quenched ball a manganese content varying between .80% and 1.00%. If a brine quench is used, the ball having been similarly treated, the manganese content of a one-half inch in diameter ball may vary between .40% and .60%; a one inch in diameter ball between .45% and .65% and a three inch in diameter ball between .50% and .70%. If the balls are directly water quenched after forging, the manganese content may vary between .35% and .55% for a ball one-half inch in diameter; between .40% and .60% for a ball one inch in diameter; and between .45% to .65% for a ball three inches in diameter. If the balls are oil quenched directly after forging, the manganese content may vary between .45% and .65% for a ball one-half inch in diameter; between .50% and .70% for a ball one inch in diameter; and between .55% and .75% for a ball three inches in diameter. If the balls are brine quenched directly after forging, the manganese content may vary between .30% and .50%.

for a ball one-half inch in diameter; between .35% and .55% for a ball one inch in diameter, and between .40% and .60% for a ball three inches in diameter.

- 5 The molybdenum content of the one-half inch in diameter ball varies between the same limits, no matter what type of quench is used, varying, preferably, between .10% and .20%. The same percentage of molybdenum is, preferably, used in 10 all the smaller size balls, no matter what type of quench is used, up to and including two inch in diameter balls. Balls up to and including those of five inch diameter, preferably, contain a somewhat higher percentage of molybdenum, varying 15 between the limits of .15% and .25%. In larger sizes than five inch balls the molybdenum content may be increased, so that for any quenching medium a molybdenum content of .40% to .60% is preferable for balls of ten inch diameter, for 20 example, and may run as high as .80% for the larger size balls.

The silicon content, preferably, does not vary to any extent for the different size balls, being, preferably, kept between .10% and .20% for all 25 size balls where a brine quench is used, or where a water quench is used, and between .15% and .25% for all size balls up to and including five inch in diameter balls, where an oil quench is used, and between .20% and .30% for balls larger than five 30 inch in diameter, where an oil quench is used.

Of course, the percentages of manganese and molybdenum may be varied from the ones stated herein, as well as the percentage of silicon, where balls with special characteristics may be desired, 35 as long as the variation is not too great from the extreme percentage limits given. Also, for extremely large size balls it may even be found desirable to vary the content of molybdenum and manganese above the upper limits stated.

- 40 The grinding element that results from the use of the alloys substantially as set forth, treated in the manner described herein, varies somewhat in characteristics, dependent upon the size of the ball, slug, or grinding element, that is produced. 45 In all cases a very hard fine grain structure is produced in the steel inwardly from the outer surface of the grinding ball, or element, a very substantial distance. This outer zone is of a fineness of grain and hardness, that has not been 50 previously attained in steel grinding balls of any kind. This hard, fine grained structure extends to a depth of at least one-half inch from the outer surface of the ball, even in the larger size balls, and extends to the center of the ball in the smaller 55 size balls, up to and including a ball of one inch diameter. The structure of this hard, fine grained portion of the larger balls and of the entire ball, in the case of balls of one inch or smaller in diameter, is a fine grained martensitic 60 structure.

While this fine grained martensitic structure has extremely great resistance to abrasion and great hardness and some ductility, it does not have sufficient ductility to withstand the impact, 65 that results when larger balls are dropped in the course of their travel in the ball mill, which, in mills in which larger balls are used, is often a considerable drop from the upper portion of the mill to the lower portion thereof. In order that this 70 impact may be absorbed in the ball without any danger of fracture of the ball, it is desirable that the larger grinding elements for use in ball mills have a core of different structure than the outer portion thereof, and one of the advantages of our 75 improved grinding element, due to the alloy used

and the method of treatment of the same to harden it, is that, in the larger sizes, by simple heating and quenching, the desired core of a different structure is obtained to absorb the impact resulting from the dropping of such larger balls and the prevention of fracture of the balls thereby, while at the same time providing the martensitic structure of a deep outer layer of the ball, or grinding element, which is necessary to get the long wear that makes our improved grinding element highly desirable and economical. 10

Referring to the drawing, Fig. 1 shows as adequately as is possible by means of a drawing, the internal structure of a larger size grinding ball, made in accordance with our invention, and Fig. 2 shows the internal structure of a smaller size grinding ball, made in accordance with our invention. The type of grinding ball shown in Fig. 1 is that of the grinding balls larger than one inch in diameter, and that shown in Fig. 2 of grinding 20 balls of one inch in diameter and smaller.

The fineness of the grain of the grinding ball is necessarily shown somewhat diagrammatically, but referring to the grinding ball shown in Fig. 1, a zone or layer of hard very fine grained 25 martensitic steel is shown at 3, extending from the outer surface 4 of the ball to a fairly well defined point 5, spaced inwardly substantially a uniform distance from the outer surface 4, at which a coarser structure begins, which extends to the center 6 of the ball. This coarser structure is made up of troostite and sorbite, and is of considerably coarser grain than the outer martensitic structure 3. The inner core portion, designated generally by the numeral 7, 30 extending from the center 6 outwardly to substantially the point 5, is, however, finer grained than any portion of a hardened carbon-manganese ball, except, possibly, a very thin skin-coat adjacent the outer surfaces of such a carbon 40 manganese steel alloy ball. It has no crevices or cracks therein of a decided character, as are found in a carbon-manganese steel ball, both in the hardened outer thin skin-coatlike zone and the inner portion thereof, which is of very coarse 45 grain, as compared with the coarsest grain portion of the core 7. There is an intermediate zone in the larger size balls, such as shown in Fig. 1 of the drawing, that contains a mixed structure that appears to be partially of the character of the inner portion of the core 7 and partially martensitic, like the outer hard fine grained portion 3. This zone is not of any great 50 depth, but consists of martensite and troostite, or martensite, troostite and sorbite.

The presence of the molybdenum in the alloy appears to be responsible for the fact that a grinding ball of either the character shown in Fig. 1, or the character shown in Fig. 2, will not lose its hardness and fine grain structure, if used under relatively high temperature conditions. Fig. 2, of course, shows a grinding element that is made up of the fine grain, hardened martensitic structure 3 from the outer surface 8 thereof to the center 9 thereof, being of a homogeneous character throughout.

The greater percentage of carbon is provided in the larger size balls, in order to obtain the desired hardness of the outer zone 3 thereof.

The point at which the change from beta to gamma iron, or vice versa, takes place, is, of course, raised by increasing the molybdenum content, and this is desirable for larger size grinding members, as the temperature to which the ball, or other grinding member, is raised be- 75

fore quenching can thus be increased to obtain a more thorough solution of the carbon, manganese and molybdenum in the iron, and at the same time obtain the desired fine grain structure. The quenching time is increased as the size of the balls increases, to permit withdrawal of the larger grinding elements at substantially the same temperature as the smaller ones, this being, of course, necessary because of the larger 10 mass of the larger balls.

We have found that balls up to two inches in diameter may be cooled slowly in the air after quenching to obtain the desired rate of cooling, while those that are of a diameter above two 15 inches, and including those four inches in diameter, are run into a furnace that is operated at a temperature of 400 degrees F. immediately after quenching, to prevent too rapid cooling, being preferably, kept in such furnace for about 20 half an hour, after which the same are slowly cooled in the air. Balls of larger diameter than four inches are run into a furnace operated at a temperature of 500 degrees F. immediately 25 after quenching, and kept in such a furnace for about half an hour, after which the same are slowly cooled in the air. The retardation of the cooling prevents the creation of internal stresses in the grinding elements that might cause breakage.

30 Grinding elements made in accordance with our invention have a much greater hardness, except for extremely small grinding elements, than the ordinary carbon-manganese alloy grinding balls that have been previously used. A comparison 35 between forged carbon-manganese grinding balls and our molybdenum alloy grinding balls, also forged, and both made according to the best known practice, and similarly heat treated and quenched, shows, upon hardness tests being 40 made of said balls at the surface thereof and at the center thereof, that balls up to and including those one inch in diameter are of the same hardness in the center as at the wearing surface, both when made of the carbon-manganese alloy 45 steel previously used, and when made by our improved method of the molybdenum alloy steel that we employ, but that the hardness of the balls made in accordance with our invention is greater for all sizes of balls than the carbon- 50 manganese alloy balls, and that the larger the ball the greater the difference. Thus, for a one-half inch ball the carbon manganese steel ball has a Rockwell C scale hardness of 64, or 700 Brinell, at the surface thereof, and also at the 55 center thereof, while our improved grinding element has a hardness at the surface and center thereof of 65 Rockwell C scale, or 720 Brinell. A one inch ball of carbon-manganese steel alloy has a Rockwell C scale hardness of 63 both at the 60 surface and the center thereof, or 680 Brinnell, while a one inch ball made in accordance with our invention has a hardness of 66 Rockwell C scale at both the surface and the center thereof, or 750 Brinell.

65 The use of our improvements in a grinding element has the advantage over the ordinary carbon-manganese alloy forged ball, that the hardness toward the center of our improved ball does not vary to any extent from that at the 70 surface until considerably larger sizes are encountered, while the hardness of a carbon-manganese steel ball decreases very perceptibly in the center, as well as on the surface thereof after the diameter increases above one inch. 75 Thus a two inch carbon-manganese steel grind-

ing ball has a hardness of only 58 Rockwell C scale, or 610 Brinell, at the surface thereof, and a hardness of only 38 Rockwell C scale, or 370 Brinell at the center thereof, whereas our improved ball of the alloy herein described, two inches in diameter, has a hardness at the surface of 64 Rockwell C scale, or 700 Brinell, and 50 Rockwell C scale or 510 Brinell at the center. A three inch ball of carbon-manganese steel alloy has an outer surface hardness of 56 Rockwell C scale, or 580 Brinell, and a center hardness of 37 Rockwell C scale, or 360 Brinell, whereas a ball of three inches in diameter made in accordance with our invention has a surface hardness of 63 Rockwell C scale, or 680 Brinell, and a center hardness of 46 Rockwell C scale, or 460 Brinell.

It will thus be noted that while the center of the three inch ball is considerably less hard than that of the two inch ball in the case of our improved grinding ball, the surface hardness is substantially the same, and this hardness extends inwardly a very substantial distance from the surface, whereas in the case of the carbon-manganese alloy it does not extend inwardly any appreciable distance, but the hardness begins decreasing rapidly from the outer surface toward the center of the ball. While the difference in hardness between a ball made in accordance with our invention and the ordinary carbon-manganese steel balls is not as great for the larger size balls as for those between one inch and three inches in diameter, yet the larger size balls are harder both on the surface and at the center thereof, when our improved molybdenum alloy steel and method of treatment is used, than when the ordinary carbon-manganese steel is used. Thus a five inch ball of carbon-manganese steel has an exterior hardness of 50 Rockwell C scale, or 510 Brinell, and a center hardness of 30 Rockwell C scale, or 300 Brinell, while a five inch ball made in accordance with our invention has a surface hardness of 53 Rockwell C scale, or 540 Brinell, and a center hardness of 40 Rockwell C scale, or 390 Brinell.

The average hardness, obtained by testing at regular spaced intervals between the outer surface and the center, of balls made in accordance with our invention and in accordance with previous practice for carbon-manganese steel grinding balls, shows that our improved grinding ball for all sizes, has an average hardness, from the outer surface to the center thereof, that is much greater than that of the carbon-manganese steel ball. Thus a ball of one-half inch diameter of carbon-manganese steel has an average hardness of 64 Rockwell C scale, or 700 Brinell, and our improved ball of the same diameter has an average hardness of 65 Rockwell C scale, or 720 Brinell. A one inch ball of carbon-manganese steel has an average hardness of 63 Rockwell C scale or 680 Brinell, while our improved ball of the same size has an average hardness of 66 Rockwell C scale, or 750 Brinell. A 65 two inch carbon-manganese ball has an average hardness of 53 Rockwell C scale, or 540 Brinell, while a two inch ball of our manufacture has an average hardness of 63 Rockwell C scale or 680 Brinell. The three inch carbon-manganese steel ball has an average hardness of 47 Rockwell C scale, or 470 Brinell, while a ball of our manufacture, three inches in diameter, has an average hardness of 62 Rockwell C scale, or 670 Brinell, and a five inch carbon- 75

manganese steel ball has an average hardness of 36 Rockwell C scale, or 350 Brinell, and our improved ball five inches in diameter has an average hardness of 43 Rockwell C scale, or 420 Brinell.

It is obvious from the above that we have provided a ball that not only has greater average hardness, but has through a large portion of its depth, a much finer grain structure than any previously manufactured steel grinding ball, and that, as a result, the wearing properties of these balls is much greater than that of steel grinding balls previously used for ball mills and similar apparatus. The effect of having the finer grained portion of considerable depth, has a very great effect on the wearing qualities of the balls. As the depth of the fine grained, substantially homogeneous outer zone is at least one-half inch, the fine grained martensitic wearing zone of a ball two inches in diameter comprises about 87.5% of the entire mass of the ball, and in the case of a three inch ball 70.4% of the entire mass of the ball, while in the case of a four inch ball it would comprise 57% of the entire mass of the ball, and for a five inch ball 48.8% of the entire mass of the ball. Comparing this with carbon-manganese steel balls, which do not have the fine grain structure, even to a depth of one-fourth inch on an average, but assuming that such maximum depth is reached by the finer grain structure in the carbon-manganese steel ball, this finer grained zone only comprises 57.8% of the entire mass of the ball in a two inch ball; only 42.1% of the entire mass in a three inch ball; only 33% of the entire mass in a four inch ball, and only 27.1% of the entire mass in a five inch ball. The wearing qualities of a ball made in accordance with our invention are accordingly increased because of this larger zone of such dense fine grained, hard, long wearing, steel, and are additionally increased above that accountable to this fact, because of the greater hardness and finer grained and denser structure of the inner portion of the larger balls, further because of the intermediate zone of considerable depth that is largely fine grained martensitic steel, and also because of the fact that there are no interior cracks or crevices of any character in our improved grinding elements, such as are found in carbon-manganese steel grinding elements previously known.

What we claim is:

1. A steel grinding element for ball mills, constituting a solid ball-like body of heat treated carbon-manganese-molybdenum steel alloy hardened throughout from its outer surface to its center of mass and having a deep wearing zone of fine grained structure extending from the outer wearing surface inwardly in a solid mass toward the geometrical center thereof, and a central solid core of coarser grained structure surrounded by and integral with said wearing zone, said alloy containing .60% to 1.10% carbon, .30% to 1.10% manganese, .10% to .80% molybdenum, not more than .30% impurities and not less than 96.7% iron.

2. A steel grinding element for ball mills, constituting a solid ball-like body of heat treated, carbon - manganese - molybdenum steel alloy hardened throughout from its outer surface to its center of mass and having a deep wearing zone of fine grained structure extending from the

outer wearing surface inwardly in a solid mass toward the geometrical center thereof, and a central solid core of coarser grained structure surrounded by and integral with said wearing zone, said alloy containing .60% to 1.10% carbon, .30% to 1.10% manganese, .10% to .80% molybdenum, not more than .30% impurities, .20% to .30% copper and not less than 96.4% iron.

3. A wear resistant, heavy steel solid ball of heat treated, carbon-manganese-molybdenum steel alloy hardened throughout from its outer surface to its center of mass and having a deep outer, hardened wearing zone of fine grained martensitic structure, and a central, solid, hardened core of coarser grained structure integral with said wearing zone, said ball having a zone between said core and outer zone of mixed fine and coarser grained structure, said alloy containing .60% to 1.10% carbon, .30% to 1.10% manganese, .10% to .80% molybdenum, not more than .30% impurities and not less than 96.7% iron.

4. A ball-like carbon-manganese-molybdenum steel alloy grinding element for ball mills, constituting a solid body hardened throughout its mass, having a deep zone of hardened fine grained martensitic structure extending from the outer wearing surface inwardly in a solid mass toward the geometrical center thereof, and a central solid hardened core of sorbitic and troostitic structure having a greater elasticity than said fine grained zone, surrounded by and integrally connected with said fine grained outer zone by a zone of mixed martensitic, sorbitic and troostitic structure, said core being of less volume than said fine grained martensitic zone, said alloy containing .60% to 1.10% carbon, .30% to 1.10% manganese, .10% to .80% molybdenum, and the balance principally iron.

5. A wear resistant heavy carbon-manganese-molybdenum steel alloy solid ball hardened throughout and having a deep outer zone of hardened fine grained martensitic structure extending from the outer wearing surface inwardly toward the geometrical center thereof, and a central solid hardened core of sorbitic and troostitic structure having greater elasticity than said fine grained zone integral with said fine grained zone, the grain and hardness of said steel alloy changing gradually through a zone of mixed martensitic, sorbitic and troostitic structure between said inner and outer zones, said alloy containing .60% to 1.10% carbon, .30% to 1.10% manganese, .10% to .80% molybdenum, and the balance principally iron.

6. An integral ball-like carbon-manganese-molybdenum steel alloy grinding element for ball mills, solid from the geometrical center thereof to the wearing surface thereof and hardened throughout its mass, said wearing surface extending over the entire periphery of said element and being uninterrupted, said element being of a hardened fine grained martensitic structure inwardly from all portions of the peripheral surface of said element to the geometrical center thereof, said alloy containing .60% to 1.10% carbon, .30% to 1.10% manganese, .10% to .80% molybdenum, and the balance principally iron.

CHARLES W. HAGENBUCH.  
FREDERICK A. MCCOY.